

Nov. 16, 1937.

C. P. McNEIL ET AL

2,099,448

ASPHALT OXIDATION

Filed Dec. 18, 1929

2 Sheets-Sheet 1



Inventors:  
Claude P. McNeil  
Samuel A. Montgomery

By Bruce K. Brown. Atty

Nov. 16, 1937.

C. P. McNEIL ET AL

2,099,448

ASPHALT OXIDATION

Filed Dec. 18, 1929

2 Sheets-Sheet 2



Inventors  
Claude P McNeil  
Samuel A Montgomery

By Bruce K. Brown ally

## UNITED STATES PATENT OFFICE

2,099,448

## ASPHALT OXIDATION

Claude P. McNeil, Whiting, Ind., and Samuel A. Montgomery, Wood River, Ill., assignors to Standard Oil Company, Chicago, Ill., a corporation of Indiana

Application December 18, 1929, Serial No. 415,096

5 Claims. (Cl. 196—74)

This invention relates to asphalt oxidation and it pertains more particularly to an apparatus and a process for preparing blown asphalt by oxidizing petroleum residua.

The object of the invention is to continuously oxidize hot petroleum residua, also called "resids", by the countercurrent application of air.

A further object is to stabilize the temperature throughout the reaction chamber and to utilize effectively the oxygen content of the air by contacting partially-oxidized asphalt with fresh air and by contacting depleted air with fresh hot residua.

A further object is to provide an asphalt oxidation tower which is divided into oxidizing and separating sections by placing the air-introducing means at a point spaced from the bottom of the tower. A further object is to provide an improved apparatus, tower structure, and arrangement of towers for effectively carrying out the improved process.

Other objects will become apparent as the description of the invention proceeds.

The invention contemplates a continuous process wherein hot petroleum residua are introduced into the top of a tower and are permitted to flow downwardly by gravity against a current of air, which is introduced at a point above the bottom of the tank and which is buoyed upwardly by the hot liquid. The gas carried below the air inlet is separated from the hot liquid near the base of the tower and is buoyed upwardly to supplement the air in agitating and oxidizing the liquid to form asphalt. The tower is preferably about thirty or forty feet tall, so that the oxygen is almost completely utilized. A series of towers can be used to obtain asphalt of any desired characteristics, the liquid being pumped from the base of one tower to the top of the next. The invention will be more clearly understood from the following detailed description.

A preferred embodiment is shown in the accompanying drawings, wherein similar parts are designated by similar reference characters, and wherein:

Figure 1 is a diagrammatic elevation partly in section showing a single tower unit and

Figure 2 is a modification showing a series of towers.

The hot residuum or hot resid may be the pipe still bottoms from petroleum distillation or may be any similar material which is capable of oxidation in the apparatus and in the manner described. In the preferred embodiment, a 15% pipe still bottoms of Mid-Continent crude is used.

The hot residuum is introduced through valved inlet pipe 10 to the top of tower 11, which, as shown in the drawings, is relatively small in diameter as compared with its height; a tall tower being required in order that the desired oxygen utilization may be secured.

The tower 11 is preferably supported by a bracket 12 mounted on the foundation 13 of concrete or other equivalent material. It is preferably surrounded by an insulating cylinder or 10 chimney 14 which is supported and spaced in any conventional manner.

The tower 11 may be provided with perforated baffle plates 15. Instead of perforated plates we may use disc-and-doughnut baffles, bubble plates 15 or any conventional means for obtaining intimate contact of the air with the descending liquid. Baffles may be entirely dispensed with when air remains intimately mixed with the asphalt without them.

Air is introduced into the tower by a valved air-supply pipe 16 and is introduced into the liquid by a diffuser 17.

When it is necessary to supply external heat, gaseous or liquid fuel may be introduced through 25 valved pipe 19 to a burner 19a which is interposed between the cylinder 14 and tower 11. Ordinarily, in a tower of sufficient height the oxygen is almost completely utilized so that there is no danger of explosion or combustion in the top 30 of the tower. As an added precaution, we provide a valved steam inlet 20 at the top of the tower so that a blanket of steam may be used above the liquid in the tower.

The oxidized material which is moving downwardly in the tower finally moves below the diffuser 17 to a quiescent portion of the tower where in the liquid asphalt is separated from the gases, that portion of the tower between the diffuser and tower bottom being in effect a separation 40 chamber.

The pipe 21 secured to the bottom of tower 11 discharges the blown asphalt through valve 22 and pipe 23 or through valve 24 and pipe 25. Pipe 23 is usually used for draining the tower, the usual outlet during continuous operation being through pipe 25 and valves 26, 27 and/or 28 to pipe 29, leading to storage tank 30. It will be observed that pipe 25 extends vertically beside tower 11 and that pipe 29 is close to and substantially parallel with it. By means of valves 26, 27, and 28, we effectively regulate the depth of liquid in tower 11.

When a small quantity is to be oxidized, it may be sufficient to use an operating depth about one-

third the height of the tower in which case valve 26 would be open to continuously discharge the oxidized product. If a greater effective depth is required in tower 11 valve 26 is closed and valve 5 27 is opened, and if a maximum depth is required valves 26 and 27 are closed and valve 28 is opened. The proper manipulation of these valves will be apparent to those skilled in the art.

Vapors are removed from the tower 11 through 10 a conduit 31 which discharges into a condenser or "steam boat" of conventional construction. Asphalt storage tank 30 is vented by pipe 32 and pipe 29 is preferably open at its upper end in order to break any siphon that might otherwise be 15 formed.

The operation of the above modification is obvious. The 15% pipe still bottoms (Mid-Continent crude) is introduced through pipe 10 preferably at a temperature between 300 and 550° F. Air 20 is introduced through diffuser 17 and it thoroughly oxidizes and agitates the residuum in its counter-current passage to the top of the tower where it is drawn off with produced and volatilized gases through conduit 31. At the base of the tower 25 the liquid is separated from the gas and is withdrawn through pipe 21 and valve 24, pipe 25 and valve 26, 27 or 28 to pipe 29 and tank 30. The use of top steam and external heat is usually 30 not necessary but these means should be incorporated in the structure to take care of unusual conditions.

Referring to Figure 2, we provide a modified tower 33 which is preferably surrounded by an insulating jacket 34, steam coils 35 or electric 35 heating means being interposed between said tower and said jacket. Air from pipe 16 may be supplied in regulated amounts through valve 36 and pipe 37 to diffuser 38 which is spaced from the bottom of tower 33 and which is designed to 40 inject air into the hot liquid in fine small bubbles for effecting agitation and oxidation.

Discharge pipe 21 leads through valve 39 and pipe 40 to a suitable storage tank or through valve 41, pump 42, and conduit 43, to the top of tower 45 which is surrounded by jacket 45 and heated by steam coils 46 or equivalent means.

Air is admitted to tower 44 through valve 47, pipe 48, and diffuser 49, which is spaced from the bottom of the tower as shown in the drawings. 50 The outlet 21 from tower 45 is connected through valve 50 and pipe 51 to a storage tank (not shown) or through valve 52 and pipe 53 to another tower similar to those hereinabove described. The depleted air, gases and vapors are 55 removed from the top of each tower through pipes 31 and 54 respectively to a suitable scrubber.

The operation of this modification is as follows: Hot residuum, which may be 15% pipe still bottoms (Mid-Continent crude), is introduced 60 through valved inlet 10 to the top of tower 33. Air from diffuser 38 blows the hot residuum to a foam whereby it is effectively agitated and oxidized. This particular form of the invention makes use of the fact that a small quantity of 65 water causes hot residuum to foam into innumerable fine bubbles. The oxidation of the asphalt probably brings about the synthesis of minute quantities of water which produces an even distribution of air and liquid by causing the liquid to 70 foam. This foam is relatively permanent in the upper portion of the tower wherein oxidation is continuously taking place throughout the extremely large surface areas of contact between 75 the gas and liquid.

The oxidized asphalt is separated from these gases in the lower portion of the tower below the diffuser, the gases from this separating chamber being buoyed upwardly to supplement the injected air in the treatment of incoming residuum. 5

If one tower treatment is sufficient, valves 41 can be closed and the blown asphalt can be removed through valve 39 and pipe 40 to storage. If further treatment is necessary valve 39 should be closed and 41 opened, the asphalt being forced 10 by pump 42 to the top of tower 44 where it undergoes further oxidation as hereinabove described. Any number of towers can be used in series in this manner.

We have not stated specific volumes of air or 15 temperatures because these features form no part of our present invention and are well understood by those skilled in the art. The rate of feed of residuum may be regulated to introduce a volume equivalent to the volume of the tank in one hour 20 when the reaction temperature is about 550° F. or we may introduce that volume in two hours when the temperature is 450 to 500° F., using about 10 or 15 cubic feet of air per gallon of 25 residuum treated. The rate of flow of residuum, rate of introduced air, and temperatures are dependent upon the charging stock and upon the finished product desired. Our invention is applicable to all variations of these conditions.

While we have described certain preferred 30 embodiments of our invention, it is understood that we are not limited to the details therein set forth except as defined by the following claims:

We claim:

1. A continuous process for treating petroleum 35 base material to blow the same, which consists in causing said material to flow downwardly through an obstructed chamber, interrupting the descent of the material by collecting it into a series of progressively arranged pools within the chamber, 40 continuously introducing a volume of air into said chamber for contact with the material under treatment, withdrawing the vapors resulting from the reaction, and continuously withdrawing the asphaltic material after the same has been subjected to contact with the air.

2. The process of continuously producing blown asphalt which comprises introducing petroleum base material into a reaction zone, causing the material to be formed into a plurality of spaced 50 pools and to flow from pool to pool, introducing a stream of oxidizing gas into the zone and causing said gas to flow through the material in the pools.

3. The process of continuously producing blown asphalt which comprises introducing petroleum base material into a reaction zone, causing the material to be formed into a plurality of spaced 60 pools and to flow from pool to pool, introducing a stream of oxidizing gas into the zone and causing said gas to flow through the material in the pools and counter-current to the flow of the material through the zone.

4. The process of continuously producing blown asphalt which comprises introducing petroleum base material into a reaction zone, causing the material to be formed into a plurality of spaced 65 pools and to flow progressively from pool to pool, introducing a stream of oxidizing gas into the 70 zone, causing the gas to flow progressively through the material in the pools counter-current to the flow of the material and withdrawing the blown asphalt from the zone.

5. The process of continuously producing blown 75

asphalt which comprises introducing petroleum base material into a reaction zone, causing the material to be formed into a plurality of spaced pools and to flow from pool to pool, introducing a stream of oxidizing gas into the zone, causing said gas to flow through the material in the pools

and controlling the temperature of the reaction zone independently of the temperatures of the petroleum base material and oxidizing gas entering the zone.

CLAUDE P. MCNEIL.  
SAMUEL A. MONTGOMERY.